# EUROPEAN PATENT SPECIFICATION

(11) **EP 0 388 090 B1**
(45) Date of publication and mention of the grant of the patent: **01.03.1995**
(21) Application number: 90302524.5
(22) Date of filing: 09.03.1990
(51) Int. Cl.: B42D 15/00

(54) **Sheet with security device**
Bogen mit Sicherheitsvorrichtung
Feuille avec dispositif de sécurité

(30) Priority: 10.03.1989 GB 8905471
(43) Date of publication of application: 19.09.1990
(73) Proprietor: THOMAS DE LA RUE & COMPANY LIMITED, London WC2N 4DE (GB)
(72) Inventor: Thomas, David William, Maidenhead, Berkshire SL6 4DJ (GB); Thoma, Max, Basingstoke, Hampshire, RC21 5JR (GB)
(74) Representative: Skone James, Robert Edmund

(56) References cited:
- EP-A- 0 156 463
- WO-A-83/00766
- CA-A- 1 116 851
- DE-A- 2 511 368
- DE-B- 2 901 150
- DE-C- 62 053
- GB-A- 315 528
- US-A- 3 366 531
- Chambers Science and Technology DIctionary, page 856 Kriminalistik 5/79, pages 211-212

## Description

The invention relates to a sheet having a security device and a method of manufacturing such a sheet.

In the field of security documents, such as banknotes and the like, there is a continuing need to incorporate security devices which prevent such security documents from being counterfeited using the increasingly sophisticated commercial printing equipment which is available.

Examples of security devices which have been used in the past include complex patterns printed on the document, optical devices such as diffraction gratings and holograms and the like.

For certain translucent papers a security feature which involves providing (usually printing) an image on both sides of the paper was developed many years ago. In one form, herein defined as a "see-through" feature, complementary images are provided on each side of the sheet precisely registered relative to one another such that when the sheet is held up to the light, the image on the back will fit exactly into spaces within the image on the front, optionally with an even unprinted margin around the perimeter. For example, each image could comprise a series of black circles the circles on one side of the sheet fitting within the spaces between circles on the other. Printing of these images is normally carried out with specialised lithographic presses which allow simultaneous front and back printing during one printing run. In this way, the tolerances applied to the design elements are typically a fraction of a millimetre and any variation caused by counterfeiting by printing both sides during different printing runs can be quickly noticed. By printing on both sides in a single impression, misregister due to variations in the dimensions of the sheet caused by change of moisture content or heating and the like are avoided.

A second feature based on the same principle is herein defined as a "print-through" feature. In this case, an image and its reverse are printed on each side of the sheet, in register, so that when the sheet is held up to the light the image on one side of the sheet substantially conceals the image on the other side of the sheet. There should be no change in appearance of the image due to mis-register. It is possible, however, for the two images to be printed in different colours which may include rainbow printing effects.

An example of a print-through feature is described in GB-A-315528.

Both see-through and print-through features have four modes of visual inspection - the first image viewed in reflected light, the image on the other side of the sheet viewed in reflected light, the composite image viewed by transmitted light as viewed from the first side and with the image on that side predominating, and finally the composite image as viewed on the other side of the sheet with the image on that side predominating. On transmissive viewing of see-through features the image on the opposite side of the sheet is seen to be in register in a genuine document. On transmissive viewing of print-through features the image on the opposite side of the sheet is not seen in a genuine document but slight misregister will reveal that the document is a counterfeit.

The printed images are generally graphical designs although alphanumeric characters which appear identical in mirror reflection may be employed. The printed images may be of the same ink colour on both sides of the sheet which will give the impression of the printing ink having penetrated through the document or the colours may be different. The print-through feature image on one side of a sheet may comprise two different printed portions on at least one side of the sheet, which may be printed in different colours. Alternatively the printed image may be formed by continuously varying colour as in security rainbow printing methods.

Security document designers frequently combine a number of individual see-through features to make composite designs with those characteristics. See-through and print-through features will sometimes be combined to give a composite overall design feature which may cover a large portion of the note eg. up to 25%.

Until now these see-through and print-through security features have best been utilised in banknotes of relatively low basis weight and have been restricted to white or near-white papers. The heavier weight papers frequently found in the more durable currencies have too high an opacity for effective use of such features. Similarly coloured papers have too high an opacity to allow ready observation of these features.

WO-A-83/00766 describes a security document, such as an identification card, having an anti-forgery device in the form of fused laminate which is very difficult to delaminate in order to obtain access to the internal printing.

CA-A-1116851 describes a method of surface treating paper webs in which part of a web is abraded.

In accordance with one aspect of the present invention, we provide a sheet comprising a paper base stock on which security printing is or will be provided, and a security device comprising a see-through or print-through feature provided on the base stock characterised in that the feature is provided in a region of the base stock which has a substantially uniform transparency and which is more transparent than a majority of the remainder of the base stock prior to the provision of security printing.

In accordance with a second aspect of the present invention, a method of manufacturing a sheet having a security device comprises providing a paper base stock on which security printing is or will be provided, the base stock having a region which has a substantially uniform transparency and which is more transparent than a majority of the remainder of the base stock prior to the provision of security printing; and providing a see-through or print-through feature in the said region.

We have proposed a new type of sheet in which a security device having a see-through or print-through feature can be provided even though a majority of the base stock itself is substantially opaque to light.

The invention is particularly applicable for use with coloured and relatively heavy security paper substrates or base stock which exhibit a high absorbance and with which see-through and print-through features have not previously been found to give satisfactory performance. These features have therefore previously been confined to lighter weight white papers. However, with the invention the advantages of these features can be used on previously unacceptable substrates. This makes the invention particularly applicable to security documents which undergo frequent use such as banknotes. The invention is applicable, however, to various types of paper based sheet substrate stock such as paper, including rag paper, paper-plastic laminates and plastic coated paper. Frequently, however, the sheet comprises rag paper to which security printing is applied to form a banknote.

Normally, the radiation with which the images can be detected is in the visible band.

The security device of the invention may be used in any suitable two side security printed documents such as banknotes, cheques including bank and travellers' cheques and passports, bonds, certificates, tickets, passes, plastic cards (such as financial cards, bank cards, credit cards, charge cards, guarantee cards, service entitlement cards), integrated circuit containing cards, identity cards, and licence documents.

The transparency of such items may be automatically measured when the item is presented for machine processing such as banknote sorting.

Preferably, the features substantially fill the region of uniform transparency although a plane perimeter region may be provided.

As already mentioned, the images printed in the region may be similar to those used conventionally to define see-through or print-through features. In addition, these features may be varied so that instead of whole evenly toned printing being employed, the images may be made from intermeshing geometric arrangements. Such arrangements include parallel spaced line patterns, for example with the space and line widths being identical, such that when the composite is viewed by transmission the lines alternately overlap to give the impression of a solid figure. Concentric circles or other curvilinear shapes may also be employed. A further alternative is an intermeshing pattern of orthogonally orientated lines of equal line and space width which when viewed by transmission give an overlapping pattern of squares having either no overlap, a single overlap or double overlap. Poor registration will cause this effect to be noticably changed. A further alternative, described in DE-C-3208204 is a periodic line or points pattern which on counterfeiting gives a moire pattern.

The images can be printed in monochrome or polychrome or a combination of the two.

The inks which may be employed are lithographic inks including coloured inks, white inks, black inks, metallic inks, optically variable inks (such as those incorporating thin film optical interference filters) and the like. Thermochromic inks, photochromic inks, fluorescing and phosphorescing inks visibly may also be employed. The inks may be employed in rainbow printing fashion.

The images may also be printed with white or colourless substances which are difficult to detect by eye but which are detectable by machine sensing, such as X-ray absorptive inks. Using such a technique the security feature will only be made viewable on an X-ray photograph.

Preferably, the step of providing a base stock comprises manufacturing the base stock such that the weight per unit area of the base stock in the region of uniform transparency is less than the weight per unit area in the majority of the remainder of the base stock. Preferably, this is achieved by the use of a watermarking technique such as by using mould or dandy roll methods but in which there is substantially no variation in transmission to radiation within the region.

As an alternative, for relatively thin sheets, the majority of the base stock can be made substantially more opaque than the region to carry the images using dyes and the like. In a further alternative, such reduction in transparency may be achieved by methods of electroless deposition of metals as taught in JP63219694A (Dai Nippon Printing KK) in which the metal deposits inside the paper without discoloration.

For a mould-made watermarked white paper, if the non-watermarked areas have an average relative transmission of 1.00, then the planar region in which the security device is provided preferably has a relative transmission of 1.05 to 1.25, most preferably 1.10 to 1.20. The shadow areas of graphical watermarks in such watermark papers may be in the range of 0.95 to 0.65, preferably 0.90 to 0.80. A particular example of a mould marked paper (prior to any printing) had a relative transmission of 1.00 in its unwatermarked areas, a maximum relative light transmission of 1.17 in the highlights and a minimum of 0.85 in the shadow areas of the graphical watermark.

For a dandy roll made watermarked white paper, the relative planar region transmissions which are preferred are similar to that for a mould-made watermarked white paper. A particular example of a dandy roll marked paper had a relative transmission of 1.00, a maximum relative light transmission of 1.17 in the highlights and a minimum of 0.89 in the shadow areas of the graphical watermark.

The variation in transmission of the unwatermarked areas prior to printing will normally be within 2%.

It should be understood that the reference above to "watermarked" paper is simply to indicate that the region in which the security device is provided has been manufactured using a watermarking technique although the region created to carry the images has a substantially uniform or even transparency.

In addition to this region, however, it is preferable if the sheet also includes a conventional (ie. graphical) watermark. This graphical watermark should be separate from the region having the security device and may be made in any conventional manner, typically the same manner as that used to make the security device region but additionally imparting a variation in the translucency of the paper. For example, there may be a mould-made mark which is a three dimensional image created within the body of the paper during the manufacturing process. It consists of a controlled variation of paper weight on a small scale which permits more or less light to pass through the paper forming areas of light and shadow which make up the graphical watermark image.

Typically, the region containing the security device will have an area of between 0.4 and 5cm² and although generally will be separate from other graphical watermark features, it could form part of a larger composite watermark. Areas greatly in excess of 5cm² are undesirable less the strength of the document is compromised.

In general, the region containing the security device will have a reduction in opacity of typically up to 40% of the average opacity of the sheet. This figure may be greater, that is the contrast between the general background areas of the sheet and the security device region may be greater if the base is itself coloured.

The process for printing the see-through or print-through features is normally twin offset lithographic although twin dry offset lithography and twin intaglio may be used. In order to achieve the precise register the image component on one side of the sheet is printed at the same time at its counterpart on the other side of the sheet. Thus the two components are applied during one printing impression, not from separate impressions even during the same pass through the printing press. The combination of lithography and intaglio will not normally give sufficient register to be practicable.

The planar watermarked area for use with these features must be even in translucency over the area of the feature with which it is designed to be used. Conventional watermarking of banknote and similar security paper causes many deliberate changes in translucency in order to depict the graphical watermark. The areas of given high translucency in conventional watermarks are generally too small for use with see-though and print-through features. In some cases, the region containing the see-through and print-through feature will be on its own, in others it may abut or be contained within a conventional graphical watermark.

Normally, the region containing the see-through or print-through feature will wholly contain the feature and leave a margin to allow for variation in register between the region and the feature. This is not however essential. Thus for example within a large conventional see-though or print-through feature there may be contained a feature according to the invention. The region incorporating this feature fits inside the conventional feature but sufficiently circumscribes the printing which is to be viewed in combination with the region. The overall effect of a localised feature according to the invention, which is contained within a larger area of see-through and/or print-through printing is to create a highlight area.

A security document such as a banknote may contain a selection of see-through and print-through features and individual design elements may include portions of both.

In the case where the security device region is made more transparent to radiation using a watermarking technique, account must be taken of the fact that the watermarking process gives less precise register than that achievable by double sided precision register lithographic printing. In view of this, the region contained in the security device will normally be made larger than the images themselves, typically by 3mm in each direction. The registration of the security device region and the images need not therefore be as accurate as between the images themselves.

A further advantage of making use of the watermarking technique is that counterfeiting is made more difficult by combining this technique with double sided precision lithographic printing.

The final registration between the images on each side of the sheet should fall within a tolerance of 0.1mm.

If the planar region is made by changing the basis weight of the paper locally, then it is desirable that this area of reduced weight does not extend over the edge of the sheet having the security device in order not to reduce the durability of the document.

In accordance with a third aspect of the present invention, security printable paper base stock comprises a region having a size sufficient to contain a see-through or print-through security feature, and having a substantially uniform transparency which is more transparent than a majority of the remainder of the base stock prior to the provision of security printing, wherein the substantially uniform transparency region was created during manufacture of the base stock and has a weight per unit area less than the weight per unit area in the majority of the remainder of the base stock. For example the stock may comprise banknote paper and may include, separate from the transparent region, one or more of a security thread, a graphical watermark, security fibres, and planchettes.

The base stock may include a sheet having at least twelve such regions and advantageously forms a roll having at least 1000 such regions.

Some examples of banknotes according to the invention will now be described with reference to the accompanying drawings, in which:-
Figure 1 illustrates one face of a banknote showing a watermark region and a region of even translucency;
Figure 2 illustrates one image of a combined see-through and print-through device;
Figure 3 illustrates the other image of the device of Figure 2;
Figure 4 illustrates the appearance of the device of Figures 2 and 3 when viewed with transmitted light;
Figure 5 illustrates the device of Figures 2 to 4 on the banknote of Figure 1;
Figure 6 illustrates another banknote having a print-through device; and,
Figures 7A and 7B illustrate respectively a cross-section through a partially printed banknote and a graph showing transmittance along the cross-section.

Figure 1 illustrates a banknote 1 containing a conventional graphical watermark 2 illustrated in outline and an area of even transparency 3.

Figure 2 represents the front view of the portion of a combined see-through and print-through device (not shown in Figure 1) which is printed on the front of the banknote 1 in the area 3 and in which the black areas are printed areas. This consists of a perimeter outline of a figurine 4, background shading 5 and an overall perimeter 6A. It is all contained within the area of even transparency 3 (not shown in Figure 2).

Figure 3 represents the view of the other portion of the device, printed on the back of the banknote 1 and viewed from that aspect. It is similarly contained within the area of even transparency 3 (not shown in Figure 3). It consists of a solid figurine 7, which may be rainbow printed, within an unprinted background 8 and confined by a perimeter 6B of the same dimensions as that in Figure 2.

Figure 4 represents the front view of the device when inspected by transmitted light. Within the area of even transparency 3 (not shown in Figure 4) is located the composite device. The figurine is revealed to be in such accurate register that it fits within the confines of the front printed portion and is surrounded by an even unprinted margin 9. This illustrates the see-through feature.

The perimeters of the portions 6A and 6B of the two printings constituting the device are printed in such accurate register that they overlap to form perimeter line 10 which has exactly the same dimensions as components 6A and 6B. This forms the print-through feature. From inspection of the device in transmitted light it is not obvious to the casual viewer that the line 6B is behind 6A.

Figure 5 shows the relative position of the device within the final banknote as viewed by transmitted light.

Figure 6 represents the appearance from the front and by transmitted light of a similar device 11 which is entirely a print-through device, with the elements being composed in similar manner to the previous example, but with the entire element being printed in register on both sides of the paper. In this instance the mirror image of the design 11 shown in Figure 6 as being on the front of the note is printed on the back in absolute register.

Figure 7A shows the banknote 1 provided with the area of even transparency 3 in which is printed a figurine 2 similar to the figurine 7. The banknote 1 has been further provided, by means of printing, with a solid figurine 13 elsewhere in the majority of the sheet. The light transmittance through the partly printed document is thus characterised by four values as shown in Figure 7B. Value A is the light transmittance through the majority of the sheet; Value B is the light transmittance through the area of even transparency 3; Value C represents the light transmittance through the area provided with the solid figurine 13; and Value D represents the light transmittance through the area of even transparency 3 provided with the solid figurine 12.

The light transmittance measurements were made with the light source on the same side as the solid printed figurines 12 and 13 and detection on the side remote from the figurines. The contrast between print and paper when the print is viewed through the paper may be defined in terms of these four values. Contrast P representing the print contrast for the solid figurine 13 printed on the majority of the sheet may be defined as Value A minus Value C. Similarly Contrast T representing the print contrast for the solid figurine 12 printed in the area of greater transparency 3 may be defined as Value B minus Value D. The increase in contrast represented by the increase of Contrast T over Contrast P is thus a measure of the improvement in the clarity of a see-through feature of the invenion.

### Example 1

A white sheet of paper of approximately 85 gsm was made on a laboratory sheet former. An area of greater transparency was provided during the forming of the sheet. The sheet was printed with a suitable solid image using black ink in the area of the greater transparency and elsewhere on the majority of the sheet. Light transmission measurements calculated from transmission densitometer readings gave the characteristic values as described above of Value A = 31.4%, Value B = 47.1%, Value C = 1.8% and Value D = 3.7%. Thus we may calculate Contrast P = 29.6% and Contrast T = 43.4%, an improvement of 13.8% in print contrast.

### Example 2

A white sheet of paper of approximately 95 gsm was formed and printed as described in Example 1. Characteristic light transmission levels were Value A = 25.7%, Value B = 41.2%, Value C = 7.8% and Value D = 11.6%. The relevant print contrast values are thus Contrast P = 17.9% and Contrast T = 29.6%, an improvement in print contrast of 11.7%.

### Example 3

A pink coloured sheet of paper of approximately 95 gsm was formed and printed as in Example 1. Characteristic light transmission levels were Value A = 12.9%, Value B = 30.9%, Value C = 3.5%, and Value D = 7.2% giving print contrasts of Contrast P = 9.4% and Contrast T = 23.7%, an improvement of 14.3%.

## Claims

1. A sheet (1) comprising a paper base stock on which security printing is or will be provided, and a security device comprising a see-through or print-through feature provided on the base stock characterised in that the feature is provided in a region (3) of the base stock which has a substantially uniform transparency and which is more transparent than a majority of the remainder of the base stock prior to the provision of security printing.

2. A sheet according to claim 1, wherein the feature is printed using a white or colourless substance which is detectable by machine sensing.

3. A sheet according to claim 1 or claim 2, further comprising a graphical watermark separate from the region (3) having the security device.

4. A sheet according to any of the preceding claims, wherein the region containing the security device has an area between 0.4 and 5cm².

5. A sheet according to any of the preceding claims, wherein the region containing the security device has a reduction in opacity relative to the remainder of the sheet in the absence of applied ink of up to 40% of the average opacity of the sheet.

6. A sheet according to any of the preceding claims, wherein the base stock is provided with security printing.

7. A sheet according to any of the preceding claims, wherein the feature is printed on the base stock.

8. A method of manufacturing a sheet having a security device, the method comprising providing a paper base stock on which security printing is or will be provided, the base stock having a region which has a substantially uniform transparency and which is more transparent than a majority of the remainder of the base stock prior to the provision of security printing; and providing a see-through or print-through feature in the said region.

9. A method according to claim 8, wherein the step of providing a base stock comprises manufacturing the base stock such that the weight per unit area of the base stock in the region of uniform transparency is less than the weight per unit area in the majority of the remainder of the base stock.

10. A method according to claim 8 or claim 9, wherein the feature is printed on the base stock.

11. A method according to any of claims 8 to 10, wherein the region is formed using a watermarking process.

12. Security printable paper base stock comprising a region having a size sufficient to contain a see-through or print-through security feature, and having a substantially uniform transparency which is more transparent than a majority of the remainder of the base stock prior to the provision of security printing, wherein the substantially uniform transparency region was created during manufacture of the base stock and has a weight per unit area less than the weight per unit area in the majority of the remainder of the base stock.

13. Stock according to claim 12 which comprises banknote paper.

14. Stock according to claim 12 or claim 13, the stock including one or more of a security thread, a watermark, security fibres, and planchettes.

15. Stock according to any of claims 12 to 14, wherein the region has an area of between 0.4 and 5cm².

16. Stock according to any of claims 12 to 15, the stock having at least twelve such regions.

17. A roll of paper stock according to claim 16, the roll having at least 1000 such regions.

18. A sheet having a security device according to any of claims 1 to 7 manufactured from paper stock according to any of claims 12 to 17.

## Patentansprüche

1. Bogen (1) mit einem Papier-Grundmaterial, auf dem ein Sicherheitsabdruck vorgesehen ist oder wird, und einer Sicherheitsvorrichtung mit einem Durchsichts- oder Durchdruck-Merkmal, das auf dem Grundmaterial vorgesehen ist, dadurch gekennzeichnet, daß das Merkmal in einem Bereich (3) des Grundmaterials vorgesehen ist, der eine weitgehend gleichförmige Lichtdurchlässigkeit hat und lichtdurchlässiger als ein größerer Teil des Restes des Grundmaterials vor der Ausbildung des Sicherheitsabdrucks ist.

2. Bogen nach Anspruch 1, bei dem das Merkmal mittels einer weißen oder farblosen Substanz gedruckt ist, das durch maschinelle Abtastung nachweisbar ist.

3. Bogen nach Anspruch 1 oder Anspruch 2 mit einem graphischen Wasserzeichen, das von dem die Sicherheitsvorrichtung aufweisenden Bereich (3) getrennt ist.

4. Bogen nach einem der vorstehenden Ansprüche, bei dem der die Sicherheitsvorrichtung aufweisende Bereich eine Flache zwischen 0,4 und 5 cm² hat.

5. Bogen nach einem der vorstehenden Ansprüche, bei dem der die Sicherheitsvorrichtung aufweisende Bereich eine gegenüber dem übrigen Teil des Bogens verringerte Opazität bei Abwesenheit von aufgebrachter Farbe von bis zu 40% der mittleren Opazität des Bogens hat.

6. Bogen nach einem der vorstehenden Ansprüche, bei dem das Grundmaterial mit einem Sicherheitsabdruck versehen ist.

7. Bogen nach einem der vorstehenden Ansprüche, bei dem das Merkmal auf dem Grundmaterial abgedruckt ist.

8. Verfahren zum Herstellen eines Bogens mit einer Sicherheitsvorrichtung, bei dem ein Papier-Grundmaterial hergestellt wird, auf dem ein Sicherheitsabdruck vorgesehen ist oder wird, wobei das Grundmaterial einen Bereich aufweist, der eine weitgehend gleichförmige Lichtdurchlässigkeit hat und lichtdurchlässiger als der größere Teil des Restes des Grundmaterials vor dem Aufbringen des Sicherheitsabdrucks ist, und bei dem ein Durchsichts- oder Durchdruck-Merkmal in dem erwähnten Bereich ausgebildet wird.

9. Verfahren nach Anspruch 8, bei dem die Herstellung des Grundmaterials derart bewirkt wird, daß das Flächengewicht des Grundmaterials im Bereich der gleichförmigen Lichtdurchlässigkeit kleiner als das Flächengewicht in dem größeren Teil des übrigen Grundmaterials ist.

10. Verfahren nach Anspruch 8 oder Anspruch 9, bei dem das Merkmal auf dem Grundmaterial abgedruckt wird.

11. Verfahren nach einem der Ansprüche 8 bis 10, bei dem der Bereich unter Anwendung eines Wasserzeichen-Ausbildungsverfahrens gebildet wird.

12. Sicherheitbedruckbares Papier-Grundmaterial mit einem Bereich, dessen Größe ausreichend ist, um ein Durchsichts- oder Durchdruck-Sicherheitsmerkmal aufzunehmen, und mit weitgehend gleichförmiger Lichtdurchlässigkeit, die größer als die des größeren Teils des restlichen Grundmaterials vor der Ausbildung des Sicherheitsabdrucks ist, wobei der Bereich mit weitgehend gleichförmiger Lichtdurchlässigkeit während der Herstellung des Grundmaterials erzeugt wurde und ein Flächengewicht hat, das kleiner als das des größeren Teils des restlichen Grundmaterials ist.

13. Material nach Anspruch 12, das Banknotenpapier aufweist.

14. Material nach Anspruch 12 oder Anspruch 13, das wenigstens einen Sicherheitsfaden, ein Wasserzeichen, Sicherheitsfasern und Planchetten (Metallplättchen) aufweist.

15. Material nach einem der Ansprüche 12 bis 14, bei dem der Bereich eine Fläche zwischen 0.4 und 5 cm² hat.

16. Material nach einem der Ansprüche 12 bis 15, das wenigstens zwölf derartige Bereiche aufweist.

17. Rolle aus Papiermaterial nach Anspruch 16, die wenigstens tausend solche Bereiche aufweist.

18. Bogen mit einer Sicherheitsvorrichtung nach einem der Ansprüche 1 bis 7, der aus einem Papiermaterial nach einem der Ansprüche 12 bis 17 hergestellt ist.

## Revendications

1. Feuille (1) comprenant une matière de base de papier sur laquelle une impression de sécurité est formée ou est destinée à être formée, et un dispositif de sécurité comprenant une caractéristique de transmission de lumière ou de transmission d'impression, placé sur la matière de base, caractérisée en ce que la caractéristique est formée dans une région (3) de la matière de base qui a une transparence pratiquement uniforme et qui est plus transparente que la majorité du reste de la matière de base avant l'application de l'impression de sécurité.

2. Feuille selon la revendication 1, dans laquelle la caractéristique est imprimée avec une substance blanche ou incolore qui peut être détectée par détection par une machine.

3. Feuille selon la revendication 1 ou 2, comprenant en outre un filigrane graphique séparé de la région (3) ayant le dispositif de sécurité.

4. Feuille selon l'une quelconque des revendications précédentes, dans laquelle la région contenant le dispositif de sécurité a une surface comprise entre 0,4 et 5 cm².

5. Feuille selon l'une quelconque des revendications précédentes, dans laquelle la région contenant le dispositif de sécurité présente une réduction d'opacité par rapport au reste de la feuille, en l'absence d'encre appliquée, qui peut atteindre 40 % de l'opacité moyenne de la feuille.

6. Feuille selon l'une quelconque des revendications précédentes, dans laquelle la matière de base est munie d'une impression de sécurité.

7. Feuille selon l'une quelconque des revendications précédentes, dans laquelle la caractéristique est imprimée sur la matière de base.

8. Procédé de fabrication d'une feuille ayant un dispositif de sécurité, le procédé comprenant la disposition d'une matière de base de papier sur laquelle une impression de sécurité est formée ou est destinée à être formée, la matière de base ayant une région qui a une transparence sensiblement uniforme et qui est plus transparente que la majorité du reste de la matière de base avant l'application de l'impression de sécurité, et l'application d'une caractéristique de transmission de lumière ou de transmission d'impression dans ladite région.

9. Procédé selon la revendication 8, dans lequel l'étape de disposition d'une matière de base comprend la fabrication de la matière de base de manière que la masse par unité de surface de la matière de base dans la région de transparence uniforme soit inférieure à la masse par unité de surface de la plus grande partie du reste de la matière de base.

10. Procédé selon la revendication 8 ou 9, dans lequel la caractéristique est imprimée sur la matière de base.

11. Procédé selon l'une quelconque des revendications 8 à 10, dans lequel la région est formée par le procédé de fabrication d'un filigrane.

12. Matière de base de papier qui peut recevoir une impression de sécurité, comprenant une région ayant une dimension suffisante pour qu'elle puisse contenir une caractéristique de sécurité par transmission de lumière ou transmission d'impression, et ayant une transparence pratiquement uniforme, cette région étant plus transparente que la plus grande partie du reste de la matière de base avant l'application de l'impression de sécurité, dans laquelle la région de transparence pratiquement uniforme a été créée pendant la fabrication de la matière de base et a une masse par unité de surface qui est inférieure à celle de la majorité du reste de la matière de base.

13. Matière selon la revendication 12, qui est un papier de billet de banque.

14. Matière selon la revendication 12 ou 13, comprenant un ou plusieurs éléments parmi un fil de sécurité, un filigrane, des fibres de sécurité et des gaufrages.

15. Matière selon l'une quelconque des revendications 12 à 14, dans laquelle la région a une surface comprise entre 0,4 et 5 cm².

16. Matière selon l'une quelconque des revendications 12 à 15, ayant au moins douze régions.

17. Rouleau de matière de base de papier selon la revendication 16, ayant au moins mille régions.

18. Feuille ayant un dispositif de sécurité selon l'une quelconque des revendications 1 à 7, fabriquée à partir d'une matière de base de papier selon l'une quelconque des revendications 12 à 17.
